

# United States Patent Office

2,711,393

Patented June 21, 1955

1

3711393

## THICKENED LUBRICANTS

**Everett C. Hughes, Shaker Heights, and Ernest C. Miller, Maple Heights, Ohio, assignors to The Standard Oil Company, Cleveland, Ohio, a corporation of Ohio.**

No Drawing. Application August 4, 1951,  
Serial No. 240,452

9 Claims. (Cl. 252—28)

This invention relates to a water-resistant, thickened lubricant in which the thickening agent is an inorganic substance.

Mineral lubricating oils are the most commonly used lubricants. Although they are available in various viscosity grades, they all possess flow properties which do not adapt them for many lubricating needs where a lubricant must adhere to the parts to be lubricated. For this reason, many proposals have been made for thickening the oils so that they will adhere to the surfaces to be lubricated, such as a wheel bearing.

A wide variety of materials has been proposed for addition to lubricating oils for thickening them. One of the materials most commonly used is soap, and soap thickened oils comprise the general class known as greases.

There are two general types of greases, those made with a calcium base soap and those made with a sodium base soap. The so-called soda base greases have relatively good temperature susceptibility properties, that is, they retain their thickened properties at reasonably elevated temperatures. However, they deteriorate readily in the presence of water, presumably because the soda base soap is very soluble in water and the solution of the soap in water emulsifies with the oil. Greases made with a calcium soap, on the other hand, have better resistance to water, presumably because the calcium soaps are water insoluble. Calcium soap base greases, however, lose their consistency or thin out at elevated temperatures, presumably because the calcium soap becomes soluble in the oil as the temperature increases.

None of the common soap base greases are entirely satisfactory with respect to both the property of maintaining good consistency at high temperatures and resisting deterioration in the presence of water.

It has also been proposed heretofore (see Patent No. 2,260,625) to prepare a thickened lubricant by combining oil with an aerogel of a material not compatible with the oil, such as silica. These aerogel-thickened lubricants have excellent temperature susceptibility properties in that they maintain their consistency at relatively high temperatures. Thus it is possible to obtain excellent penetration values up to 300° F.; this is not possible with the usual soap base greases. The aerogel greases, however, are particularly susceptible to deterioration in the presence of water. In this respect they are more vulnerable than the soap base greases, as will be seen in the tables set forth hereinafter.

As will be explained hereinafter, the aerogel may be wetted by either oil or water, but is preferentially wet by water, and in the presence of water the oil phase leaves the aerogel and the thickening properties are at once destroyed.

In accordance with this invention, it has been discovered that a lubricating oil thickened with a non-abrasive, inorganic thickening or gelling agent, and particularly finely divided silica, a silica aerogel being illustrative, may be rendered resistant to water by including in the composition a surface active, oil-dispersible, water-

2

insoluble alkyl alkyloil imidazoline of the general structure:



where R is an alkylol group and R' is an alkyl or alkylene group.

These compounds are prepared by reaction of aliphatic acids and hydroxy diamines followed by cyclization, in the following way:



Hydroxy diamines in which R is of from 1 to about 6 carbon atoms, such as hydroxyethyl and hydroxyisopropyl, are readily available and are preferred. The chain length for R is dependent upon the alcoholic (polar) character of the group; the larger the number of carbon atoms, the more the group takes on the character of a hydrocarbon and loses its alcoholic character. An upper limit of about 18 carbon atoms for R is indicated by this requirement. R', which is derived from an acid, can have from 11 to 21 carbon atoms, such as undecyl, tridecyl, pentadecyl, undecenyl, heptadecyl and heptadecenyl. The thickened lubricant so prepared has excellent temperature susceptibility properties which are characteristic of the silica aerogel greases, and in addition is highly resistant to deterioration by water.

The presence of the alkyl alkylol imidazoline also does not markedly affect the consistency of the thickened lubricant, i. e., the amount of the inorganic gelling agent to impart a given consistency to the thickened lubricant is not materially modified. Furthermore, the inclusion of the alkyl alkylol imidazoline will not effect a change in the consistency of the thickened lubricant upon storage. This is to be contrasted with other materials which impart a lower initial consistency or a lower consistency on standing.

Due to the inorganic nature of the gelling agent, the thickened lubricant has excellent storage stability. This is to be contrasted with the heat susceptibility and deterioration of fatty materials in soap.

The preparation is simple and readily adaptable to continuous operation as contrasted with the involved grease-making techniques which are often considered in the industry as an art.

The oil stock used in making the thickened lubricant may be widely varied as contrasted with present grease-making requirements in which the oil in many cases is critical to meet certain specifications.

5. In addition, the avoidance of the use of soap permits the manufacturer to be independent of the supply, which is important in periods in which fats and soaps are scarce and many times of pronounced non-uniformity.

The inorganic gelling agent to be used in making the thickened lubricant in accordance with this invention may be any inorganic material which forms a gel with a lubricating oil and which is so finely divided as to be non-abrasive. The preferred materials are the aerogels, which may be formed from any material not incompatible with oil, such as silica, alumina, and other gel-forming metal oxides.

A series of silica gels which can be used as the inorganic gelling agent of the invention are manufactured by Monsanto and marketed under the trade name "Santocel."

Santocel C is prepared from a sodium silicate solution in the following way: The solution is neutralized with sulfuric acid and then allowed to stand until the mixture

sets to form a hydrogel. The by-product sodium sulfate is washed out by the repeated washings with water. The continuous water phase in this hydrogel is then replaced by continued washing with alcohol until an alcogel is formed. In order to remove the liquid phase without a collapse of the gel structure, the alcogel is placed in an autoclave which is then heated above the critical temperature of the alcohol and the pressure is allowed to increase to a point above the critical pressure of the alcohol. The vent valve is then opened and the alcohol allowed to escape. Under these conditions, the silica gel structure remains practically undisturbed and the liquid phase of the gel is replaced with air. The material is then reduced in particle size by blowing it through a series of pipes containing sharp bends with jets of compressed air. Santocel C has a secondary particle size of about 3 to 5 microns.

Santocel A is prepared as set forth for Santocel C up to the point of removal of the product from the autoclave. This material is run through a continuous heating chamber where it is heated for  $\frac{1}{2}$  hour to a temperature of about  $1500^{\circ}$  F. to eliminate the last traces of volatile material. It is then broken down in a reductionizer or micronizer to a particle size of about  $\frac{1}{16}$  inch in diameter. The solids content of the original hydrogel used in preparing Santocel C is approximately 25% higher than that of Santocel A.

AR is a modification of A, differing only in that the material is reductionized to about the same particle size as C, approximately 3 to 5 microns in diameter.

ARD is a modification of AR, differing only in that ARD is densified by extracting air under vacuum, and therefore has a smaller volume than AR.

AX is an A which has not been devolatilized.

CDv is a C which has been devolatilized as set forth for Santocel A. The Santocel is reductionized before being devolatilized.

CDvR differs slightly from CDv in that the CDvR has been devolatilized just after heating in the autoclave and then reductionized. It differs from CDv in that the latter is reductionized before being devolatilized.

The primary differences between the A and C series are as follows:

1. The C's are prepared from a sodium silicate solution containing 25% more silica than the A's. Therefore, in general the A's are lighter and composed of smaller particles than the C's.

2. The A's have undergone a devolatilization step in their preparation.

The following are the bulk densities of several of the preferred silica aerogels:

Density, grams per ml.

|     |                |
|-----|----------------|
| AR  | 0.029          |
| ARD | 0.056 to 0.064 |
| C   | 0.082          |

In general, AR and ARD show superior gelling ability and the A's in general are better than the C's. Silica aerogels which have been devolatilized generally have a higher gelling efficiency than the undevolatilized aerogels.

Other types of inorganic gelling agents which may be used include a Fumed Silica marketed by B. F. Goodrich Company. It is finely divided and appears very much like an aerogel. It is made by a combustion or vaporization process, as a source of white "carbon black" for the rubber industry. The particles are several microns in size and porous in nature.

Another material is "Linde Silica Flour" marketed by Linde Air Products Co. It is very similar in physical appearance to the silica aerogel. The particle size of the silica is purported to be 0.01 to 0.05 micron and to be manufactured by burning silicon tetrachloride and collecting the combustion product on cool plates analogous to the production of carbon black. The particles are thought to be aggregates or clusters of particles rather than of sponge-like character.

Still another inorganic gelling agent known is "Ludox" silica from Du Pont, which is known as a silica sol, and silica derivatives thereof. It has a particle size of the order of 0.01 to 0.03 micron.

In preparing thickened lubricants it is necessary to remove the water from the sol and replace it with an oil. This is possible by formulating the lubricant and removing the water by flash distillation or azeotropic distillation.

No attempt is made to enumerate all of the inorganic gelling agents which will be suitable, nor to present examples of all of them since the novel aspects of the invention reside in water-proofing the lubricant rather than the use of novel gelling agents, per se.

The lubricating oil to be used in the process may have any lubricating viscosity. It may be raw oil, acid refined, or solvent refined, as required for the particular lubricating need.

The nature of the base oil has been found to make little difference in the relative consistencies of the thickened lubricants and conventionally (acid) refined oils produce slightly thicker lubricants than solvent-refined oils. Excellent working stability is obtained regardless of the type of the base oil. An increase in the viscosity of the base oil, as might be expected, brings increased viscosity to the thickened lubricant, and minimizes bleeding. The change is relatively small and fairly linear. The viscosity of the oil does not affect the working stability of the lubricant.

The relative proportions of the inorganic gelling agent and the oil will vary somewhat depending upon the desired body in the thickened lubricant, the gelling ability of the inorganic gelling agent and the viscosity of the oil used. It has been noted, for instance, that with the Linde Silica Flour, the lubricants are somewhat harder, i. e., have a lower penetration than lubricants containing the same weight of "Santocel." Lubricants made with low viscosity oils require a somewhat larger amount of the inorganic gelling agent to give a lubricant of the same penetration. The thickened lubricant may vary in consistency from the consistency of a slightly thickened oil to a solid or semi-solid of grease-like consistency. In general, the amount of the inorganic gelling agent falls within the range of 5 to 20%, and in most cases would fall within the range of 7 to 12%.

The amount of the inorganic gelling agent, as might be expected, affects the consistency of the thickened lubricant in that an increase in its concentration brings a corresponding increase in consistency. The range is fairly linear and the amount of the gelling agent can be selected with relation to the consistency desired in view of the information in the following examples. While the difference is slight, the lubricants made with lower concentrations of gelling agent possess better working stability, while lubricants with larger amounts of gelling agent show slightly improved temperature susceptibility characteristics. The bleeding tendencies are decreased by increasing concentrations of the gelling agent.

In general, the properties of the thickened lubricants are remarkably independent of the composition variables and are not critical. The relative concentration of the gelling agent effects the most significant alteration, particularly with regard to the final consistency of the product. This permits the manufacture of thickened lubricants having a wide variety of consistencies.

The alkyl alkylol imidazoline which is included to render the thickened lubricant water resistant, is water-insoluble, oil-dispersible and surface active. The long chain alkyl group is generally recognized as imparting hydrophobic properties. The expression "oil-dispersible" includes materials which are oil-soluble. In general, the concentration of the imidazoline will vary from 0.1% to about 5%, depending upon the water stabilizing effect desired, the nature of the particular compound selected, the amount and nature of the gelling agent used, and the economics involved. A cheap compound, of course, can

be used in much larger quantities than an expensive compound, at the same total cost for the lubricant.

The composition is made simply by mixing the inorganic gelling agent, the oil and the alkyl alkylol imidazoline in any order or manner so that the imidazoline comes into intimate contact with the inorganic gelling agent.

In one embodiment, the imidazoline is incorporated with the inorganic gelling agent, for example, by dissolving the imidazoline in a solvent, such as pentane, mixing it with the gelling agent, and then evaporating the pentane. Such a treated gelling agent can be sold as an article of commerce, and dispersed in an oil when the aerogel grease is to be prepared.

Generally, the imidazoline is dispersed in the oil and the inorganic gelling agent added thereto and mixed therewith. Any simple mixing technique may be employed, and if desired the mixture may be homogenized in a colloid mill, although this is unnecessary.

The imidazoline must be uniformly distributed in the composition or on the inorganic gelling agent. For this reason the imidazoline is generally oil-dispersible or soluble—or the equivalent—soluble in some medium, which permits its application to the gelling agent.

While the invention is not to be limited to any theory or explanation, it may be of assistance in understanding the same to explain that the inorganic gelling agent is either oil-wettable or water-wettable, but it is preferentially water-wettable and has a great compatibility with water. When a lubricant thickened with an aerogel, for example, is contacted with water, the water replaces the oil in the gel and then separates from the oil. In accordance with the invention, the imidazoline, due to its surface activity, becomes attached to the silica and protects it from being wet by the water.

The imidazoline nucleus, since it possesses cationic character, is attracted to the anionic silica particles, with the result that the hydrophobic alkyl group of the molecule projects outward. Since water molecules are thus prevented from contacting the silica, the stabilizing agent, although less polar than water, is not eluted. However, the coated silica particles are easily wetted by oil since the long chain alkyl groups are oleophilic. Any mode of compounding the thickened lubricant which permits the imidazoline to come into contact with the inorganic gelling agent so as to protect it in this way, may be employed.

The composition of the invention is not limited to the oil, gelling agent, and imidazoline. Any of the materials conventionally added to lubricants and greases may be included. The expression "consisting essentially

of" as used herein is intended to refer to the components which are essential to the composition, namely, the oil, the inorganic gelling agent, and the imidazoline; and the expression does not exclude other components from the composition which do not render it unsuitable for lubrication, such materials being for instance, high polymers to modify viscosity or viscosity index, materials to impart tackiness, lubricating solids such as graphite, antioxidant additives, corrosion inhibitors of various types, sulfur, additives to render the lubricant suitable for use in gears, for cutting, grinding, etc.

The following examples illustrate preferred embodiments of the invention. Thickened lubricants made with the Amine "O," 1-β hydroxy ethyl 2-heptadecenyl imidazoline, gave good results with a small amount of the imidazoline, and for this reason Amine "O" is used in many of the examples to study the effect of other variables.

Several alkyl alkylol imidazolines of the invention in an 0.8% concentration were incorporated in a thickened lubricant formed from 8% silica aerogel (Santocel ARD)

0.8% imidazoline  
25 0.5% Paraflo  
0.5% methane base (antioxidant)  
1.0% Paratac  
0.01% dye

30 and 89.19% of a solvent extracted bright stock of 150 SSU at 210° F.

A rigorous test to determine water stability was carried out on samples of the thickened lubricants. In accordance with this test a 2 x 2 in. stainless steel plate 35 was coated with a uniform layer of the thickened lubricant, following which the coated plate was immersed in a beaker filled with tap water and boiled for a period of 60 minutes. A grease made only from oil and silica aerogel, for example, broke down immediately upon contact with the boiling water. The thickened lubricant which according to an empirical visual observation was essentially unchanged in appearance was rated "very good" or "good." If the grease separated (oil to surface, gel to bottom) it was rated "bad" or "no water stability." If some emulsification was noted, but the grease was not disintegrated, it was rated "fair."

The penetrations of the lubricants were determined using the ASTM grease penetration test in accordance with method D-217-48.

The results are reproduced in the following table:

TABLE I

| Example No.         | Additive Structure                                                                                       | Additive Oil Solu-<br>bility | Water Stability                                               | ASTM Pens |     |
|---------------------|----------------------------------------------------------------------------------------------------------|------------------------------|---------------------------------------------------------------|-----------|-----|
|                     |                                                                                                          |                              |                                                               | Unworked  | 60  |
| Lime Soap grease    | None                                                                                                     | do                           | Melts; some separation.                                       | 321       | 338 |
| Aerogel Base Grease | do                                                                                                       | Soluble                      | Bad                                                           | 221       | 238 |
| 1.                  | Armeen 10 D (Armour) Primary amine 90% C <sub>10</sub> , 3% C <sub>8</sub> , 7% C <sub>12</sub> .        | do                           | do                                                            |           |     |
| 2.                  | C <sub>12</sub> ethyl dimethyl amine<br>C <sub>12</sub> H <sub>25</sub> N(CH <sub>3</sub> ) <sub>2</sub> | do                           | do                                                            |           |     |
| 3.                  |                                                                                                          | do                           | Very poor emulsification with water sep. of oil and Santocel. | 214       | 238 |
| 4.                  |                                                                                                          | do                           | Very poor emulsification and sep. of oil and Santocel.        | 220       | 246 |

R is polypropylene

Table 1—Continued

| Example No.     | Additive Structure | Additive Oil Solubility | Water Stability                                              | ASTM Pens |     |
|-----------------|--------------------|-------------------------|--------------------------------------------------------------|-----------|-----|
|                 |                    |                         |                                                              | Unworked  | 60  |
| 5               |                    | do                      | No water stability; complete sep. of oil and Santocel.       | 233       | 250 |
| 6               |                    | do                      | No water stability; complete sep. of oil and Santocel.       | 248       | 254 |
| 7               |                    | Partially Soluble       | Bad Santocel and oil separate in 10 minutes.                 | 219       | 241 |
| 8               |                    | Soluble                 | Very good                                                    | 234       | 248 |
| 9               |                    | Not Soluble             | Bad emulsification and water separation of oil and Santocel. | 207       | 249 |
| 10              |                    | Soluble                 | Very good                                                    | 200       | 270 |
| 11              |                    | Partially Soluble       | Very poor                                                    | 238       | 247 |
| 12              |                    | Soluble                 | Very good                                                    | 233       | 254 |
| 13              |                    | do                      | do                                                           | 237       | 255 |
| 14 <sup>1</sup> |                    | do                      | Good                                                         | 234       | 248 |

<sup>1</sup> A commercial hydroxyethyl heptadecenyl imidazoline, sold under the trade name Amine "O" by the Alrose Chemical Co.

<sup>2</sup> Derived by reaction of tall oil fatty acids with the corresponding diamine, as set forth in the reaction at column 2.

As the table shows, an ordinary lime soap base grease, although conventionally regarded as water-resistant, is not water resistant by the test employed herein. This shows the severity of the test.

Examples 1 and 2 are of compounds disclosed in the art to be additives for improving the water-resistant aero-gel base greases. However, the previously accepted tests by which their water-resistance is determined are carried out at room temperature. These amines may improve water-resistance as measured by these tests, but

the table above shows they are not as effective at elevated temperatures.

The remaining examples of the table are of imidazolines. Examples 3 and 4 show the hydroxyalkyl group must be on the 1-nitrogen and that there must be both an alkylol and an alkyl group. Examples 5 and 6 show the importance of the alkylol group on the 1-nitrogen; even though there is a proper alkyl group on the 2-carbon, these compounds are not effective.

75 A comparison of Examples 7, 9 and 11 with Examples

8, 10 and 12 also shows the importance of the N-hydroxyalkyl group in making the imidazoline an effective stabilizer.

Examples 13 and 14 also are excellent additives.

In general, Table I shows that imidazolines lacking a hydroxyalkyl group on the 1-nitrogen and/or an alkyl group on the 2-carbon are ineffective, while imidazolines bearing both these groups are very effective stabilizers.

#### Examples 15 to 18

As mentioned heretofore greases made with inorganic gelling agents have better temperature susceptibility properties, e. g., they change less in consistency and penetration with a change in temperature. While it is believed this has been appreciated in the prior art because of the inorganic nature of the gelling agent, the following examples are included in order to demonstrate that the inclusion of the imidazoline does not interfere with this property. The following examples are typical and show

The superiority of the thickened lubricants made with the invention is readily apparent.

#### Examples 19 to 30

To indicate the worked and unworked penetrations and the working stability obtained with thickened lubricants made in accordance with the invention, a series of thickened lubricants were prepared, in all of which the oil was an acid refined oil having a viscosity of 300 SSU at 100° F. Each of the compositions contained 1/2% "Paraflo," a Friedel-Crafts reaction product, useful as a pour point depressant and sold by the Enjay Company, Inc., the amount of Amine "O" and the amount of gelling agent indicated in the table, and the balance was oil.

These compositions were subjected to unworked penetration tests using the ASTM grease penetration test, and were worked in accordance with the motorized ASTM worker for different number of strokes, and the results indicated in the following table:

TABLE IV

| Example No. | Gelling Agent and Amount | Amount of Amine "O" | Penetration at 77° F. After No. of Strokes Indicated |     |       |       |       |        |
|-------------|--------------------------|---------------------|------------------------------------------------------|-----|-------|-------|-------|--------|
|             |                          |                     | Unworked                                             | 60  | 2,500 | 5,000 | 7,500 | 10,000 |
| 19          | 9% Santocel C            | 1.9                 | 355                                                  | 366 | 370   | 368   | 370   | 368    |
| 20          | 10% Santocel C           | 0                   | 330                                                  | 342 | 343   | 341   | 340   | 342    |
| 21          | 12.5% Santocel C         | 1.25                | 222                                                  | 250 | 254   | 258   | 264   | 273    |
| 22          | 8% Linde Silica Flour    | 0.8                 | 333                                                  | 341 | 335   | 335   | 337   | 337    |
| 23          | 10% Linde Silica Flour   | 1.0                 | 284                                                  | 268 | 273   | 278   | 285   | 288    |
| 24          | 11% Linde Silica Flour   | 1.1                 | 198                                                  | 230 | 245   | 256   | 267   | 267    |
| 25          | 9% Santocel D            | 0.9                 | 355                                                  | 364 | 358   | 354   | 352   | 352    |
| 26          | 11% Santocel D           | 1.1                 | 240                                                  | 273 | 278   | 286   | 291   | 290    |
| 27          | 8% Santocel C            | 0.8                 | 359                                                  | 369 | 371   | 375   | 373   | 373    |
| 28          | 10% Santocel CX          | 1.0                 | 263                                                  | 298 | 310   | 309   | 309   | 311    |
| 29          | 8% Santocel A            | 0.8                 | 337                                                  | 347 | 342   | 340   | 339   | 338    |
| 30          | 11% Santocel A           | 1.1                 | 250                                                  | 268 | 265   | 264   | 262   | 269    |

the temperature susceptibility of various greases and thickened lubricants. The high temperature susceptibility index is obtained by subtracting the penetration at 77° F. from the penetration at 300° F. and dividing by the penetration at 150° F. The average temperature susceptibility index is obtained by subtracting the penetration at -4° F. from the penetration at 300° F. and dividing by the penetration at 77° F. The smaller the number in all instances, the better the temperature susceptibility.

TABLE II

| Example No. | Amount of Santocel C | Amount of Amine "O" | Amount and Nature of Other Ingredient | Nature and Viscosity of Oil Comprising Balance | Temperature Susceptibility Index |               |
|-------------|----------------------|---------------------|---------------------------------------|------------------------------------------------|----------------------------------|---------------|
|             |                      |                     |                                       |                                                | High Temp.                       | Average Temp. |
| 15          | Percent 10           | Percent 1           | 0%                                    | Solvent Extracted Oil, 300 SUS.                | 0.05                             | 0.34          |
| 16          | 12.5                 | 1.25                | 1% Paratac <sup>1</sup>               | do                                             | 0.01                             | 0.34          |
| 17          | 10                   | 1                   | 0%                                    | Solvent Extracted Oil, 175 SUS.                | 0.08                             | 0.17          |
| 18          | 10                   | 1                   | 2% Paratac <sup>1</sup>               | do                                             | 0.04                             | 0.22          |

<sup>1</sup> An isobutylene polymer sold by the Enjay Company, Inc., commonly used in compounding grease.

These above are to be compared with three conventional greases obtained upon the open market and made by well-known manufacturers. They have the following compositions and temperature susceptibility indexes:

TABLE III

| Nature of Soap | Percent of Soap | Oil            |                 | Temperature Susceptibility Index |               |
|----------------|-----------------|----------------|-----------------|----------------------------------|---------------|
|                |                 | Viscosity, SUS | Viscosity Index | High Temp.                       | Average Temp. |
| N              | 19.6            | 172            | 93.4            | 0.71                             | 1.12          |
| N              | 13.4            | 15.94          | 63              | .29                              | .93           |
| L              | 12.2            | 661.4          | 63.5            | .34                              | .84           |

In order to demonstrate further the utility of the invention, a composition was made containing 11.9% of Santocel C, 1% Amine "O," 0.9% Paraflo and the balance an acid refined oil having a viscosity of 900 SUS. This thickened lubricant was installed in the rear wheels of two Autocar tractors and the wheels were inspected

after accumulating a total of 22,322 miles. The inspection showed that the consistency of the lubricant after this period of use was very good and that the lubricant had wear resisting properties better than that of a comparable unit operating on a conventional wheel bearing grease.

General appearance of the effect of the lubrication by the thickened lubricant was entirely satisfactory

except that the bearing needed repacking as would be

expected after this mileage.

Example 32

(a) A thickened lubricant was made by mixing 10% of a silica aerogel (Santocel C) with 89% of 300 Red Oil and 1% of Amine "O."

(b) 10% of silica aerogel (Santocel C) was mixed with 85% of 300 Red Oil, 1% of Amine "O" and 4%

of Paratac (an isobutylene polymer sold by Enjay Company, Inc.) which is commonly used in conventional grease formulations to cause the grease to adhere to the surface to be lubricated.

Composition (a) was placed in the right front and left rear wheel bearings of a 1947 Mack 5-10-A tractor truck and composition (b) was used in the left front and right rear wheel bearings of the same truck. The truck was run for a period of 2½ months over a distance of 21,870 miles and inspected. The bearing rollers appeared oily by visual observation indicating good lubrication. Composition (a) was somewhat thinner, but it adhered to the bearing and there was no evidence of deterioration of the composition. Composition (b) was unchanged, and there was no evidence of deterioration. All of the bearings were in excellent condition indicating that the compositions functioned as satisfactory wheel lubricants even under severe conditions.

*Example 33*

A composition is made by mixing 5% of a silica aerogel (Santocel C) with 89.5% of an acid-refined oil having a viscosity of 300 SUS at 100° F. (300 Red Oil), 0.5% of Amine "O" as described in Example 1, and 4% of Paratac as described in Example 25(b).

*Example 34*

A composition is made from 7.5% of a silica aerogel (Santocel C), 89.75% of 300 Red Oil, 0.75% of Amine "O" and 2% Paratac.

*Example 35*

A composition is made from 10% of a silica aerogel (Santocel C), 89% of 300 Red Oil and 1% of Amine "O."

*Example 36*

A composition is made from 5% of a silica aerogel (Santocel C), 87.5% of 300 Red Oil, 0.5% of Amine "O," 4% Paratac, and 3% of a conventional extreme pressure additive.

*Example 37*

A composition is made from 7.85% of a silica aerogel (Santocel C), 82.6% of 300 Red Oil, 0.79% of Amine "O," 3.9% Paratac, and 4.85% lard oil.

Each of the above compositions was tested in a 365 B. S. center exhaust impact wrench. This machine is an air-driven impact wrench designed for tightening nuts. The main requisite for a lubricant for this type of wrench is that it be quite thin in order to keep the power loss from the drag of the lubricant as low as possible. The criteria of successful performance is an initial low torque reading and a continued low torque throughout the time of the test. The torque measurements were obtained with the wrench running free and represents the drag of the lubricant on the power output of the tool. The following table represents the initial torque, torque after two minutes and the torque after six minutes when the compositions of Examples 33 to 37 were tested in the impact wrench as compared to two soap-base greases obtained on the open market under the trade names of "#2 Roller Bearing" and "Wringer Post" which are recommended for this type of lubrication.

TABLE V

| Lubricant              | Initial Torque | Torque after 2 Minutes | Torque after 6 Minutes |
|------------------------|----------------|------------------------|------------------------|
| #2 Roller Bearing..... | 2.5            | 1.8                    | 1.6                    |
| Wringer Post.....      | 4.0            | 2.3                    | 1.8                    |
| Example 33.....        | 2.2            | 1.1                    | 0.9                    |
| Example 34.....        | 2.1            | 1.2                    | 1.1                    |
| Example 35.....        | 2.0            | 1.6                    | 1.3                    |
| Example 36.....        | 1.3.5          | 1.4                    | 1.3                    |
| Example 37.....        | 2.7            | 1.4                    | 1.3                    |

<sup>1</sup> Drops to 1.6 after 30 seconds.

Considering the initial torque and the torque after the wrench had run for various periods, the group of lubricants made in accordance with the invention as a whole, represent a marked improvement over the conventional greases of the prior art.

In order to determine further the lubricating properties of the composition, the composition of examples 33, 34, 36 and 37 were compared with the "#2 Roller Bearing" grease, in determining the horsepower loss due to grease drag on a 365 B. S. center exhaust impact wrench used in breaking bolts. Six each of  $\frac{5}{8}$ -11 and  $\frac{3}{4}$ -10 bolts were used and all threads were lubricated with a standard thread lubricant. The time required to break these bolts was recorded in seconds and the average time was taken and converted into horsepower output. The results are shown in the following table:

TABLE VI

| Lubricant              | Horsepower Output of Tool |                        |
|------------------------|---------------------------|------------------------|
|                        | $\frac{5}{8}$ -11 Bolt    | $\frac{3}{4}$ -10 Bolt |
| #2 Roller Bearing..... | .75                       | .54                    |
| Example 33.....        | .93                       | .78                    |
| Example 34.....        | .89                       | .705                   |
| Example 36.....        | .85                       | .575                   |
| Example 37.....        | 1.03                      | .705                   |

It will be seen that in all instances the horsepower output using the compositions of the invention was greater than the conventional soap-base grease recommended for this type of use.

*Examples 38 to 50*

The following imidazolines can be substituted for any of the imidazolines in the greases of the preceding examples with good results:

| Example No. | Additive Structure                                                             |
|-------------|--------------------------------------------------------------------------------|
| 38.....     | <chem>CC(C1=CC=C(C=C1)N(CCCCCCCCCCCCCCCCC)C2=CC=C(C=C2)O)C3=CC=C(C=C3)O</chem> |
| 39.....     | <chem>CC(C1=CC=C(C=C1)N(CCCCCCCCCCCCCCCCC)C2=CC=C(C=C2)O)C3=CC=C(C=C3)O</chem> |
| 40.....     | <chem>CC(C1=CC=C(C=C1)N(CCCCCCCCCCCCCCCCC)C2=CC=C(C=C2)O)C3=CC=C(C=C3)O</chem> |
| 41.....     | <chem>CC(C1=CC=C(C=C1)N(CCCCCCCCCCCCCCCCC)C2=CC=C(C=C2)O)C3=CC=C(C=C3)O</chem> |
| 42.....     | <chem>CC(C1=CC=C(C=C1)N(CCCCCCCCCCCCCCCCC)C2=CC=C(C=C2)O)C3=CC=C(C=C3)O</chem> |
| 43.....     | <chem>CC(C1=CC=C(C=C1)N(CCCCCCCCCCCCCCCCC)C2=CC=C(C=C2)O)C3=CC=C(C=C3)O</chem> |
| 44.....     | <chem>CC(C1=CC=C(C=C1)N(CCCCCCCCCCCCCCCCC)C2=CC=C(C=C2)O)C3=CC=C(C=C3)O</chem> |
| 45.....     | <chem>CC(C1=CC=C(C=C1)N(CCCCCCCCCCCCCCCCC)C2=CC=C(C=C2)O)C3=CC=C(C=C3)O</chem> |
| 46.....     | <chem>CC(C1=CC=C(C=C1)N(CCCCCCCCCCCCCCCCC)C2=CC=C(C=C2)O)C3=CC=C(C=C3)O</chem> |
| 47.....     | <chem>CC(C1=CC=C(C=C1)N(CCCCCCCCCCCCCCCCC)C2=CC=C(C=C2)O)C3=CC=C(C=C3)O</chem> |
| 48.....     | <chem>CC(C1=CC=C(C=C1)N(CCCCCCCCCCCCCCCCC)C2=CC=C(C=C2)O)C3=CC=C(C=C3)O</chem> |
| 49.....     | <chem>CC(C1=CC=C(C=C1)N(CCCCCCCCCCCCCCCCC)C2=CC=C(C=C2)O)C3=CC=C(C=C3)O</chem> |
| 50.....     | <chem>CC(C1=CC=C(C=C1)N(CCCCCCCCCCCCCCCCC)C2=CC=C(C=C2)O)C3=CC=C(C=C3)O</chem> |
| 51.....     | <chem>CC(C1=CC=C(C=C1)N(CCCCCCCCCCCCCCCCC)C2=CC=C(C=C2)O)C3=CC=C(C=C3)O</chem> |
| 52.....     | <chem>CC(C1=CC=C(C=C1)N(CCCCCCCCCCCCCCCCC)C2=CC=C(C=C2)O)C3=CC=C(C=C3)O</chem> |
| 53.....     | <chem>CC(C1=CC=C(C=C1)N(CCCCCCCCCCCCCCCCC)C2=CC=C(C=C2)O)C3=CC=C(C=C3)O</chem> |
| 54.....     | <chem>CC(C1=CC=C(C=C1)N(CCCCCCCCCCCCCCCCC)C2=CC=C(C=C2)O)C3=CC=C(C=C3)O</chem> |
| 55.....     | <chem>CC(C1=CC=C(C=C1)N(CCCCCCCCCCCCCCCCC)C2=CC=C(C=C2)O)C3=CC=C(C=C3)O</chem> |
| 56.....     | <chem>CC(C1=CC=C(C=C1)N(CCCCCCCCCCCCCCCCC)C2=CC=C(C=C2)O)C3=CC=C(C=C3)O</chem> |
| 57.....     | <chem>CC(C1=CC=C(C=C1)N(CCCCCCCCCCCCCCCCC)C2=CC=C(C=C2)O)C3=CC=C(C=C3)O</chem> |
| 58.....     | <chem>CC(C1=CC=C(C=C1)N(CCCCCCCCCCCCCCCCC)C2=CC=C(C=C2)O)C3=CC=C(C=C3)O</chem> |
| 59.....     | <chem>CC(C1=CC=C(C=C1)N(CCCCCCCCCCCCCCCCC)C2=CC=C(C=C2)O)C3=CC=C(C=C3)O</chem> |
| 60.....     | <chem>CC(C1=CC=C(C=C1)N(CCCCCCCCCCCCCCCCC)C2=CC=C(C=C2)O)C3=CC=C(C=C3)O</chem> |
| 61.....     | <chem>CC(C1=CC=C(C=C1)N(CCCCCCCCCCCCCCCCC)C2=CC=C(C=C2)O)C3=CC=C(C=C3)O</chem> |
| 62.....     | <chem>CC(C1=CC=C(C=C1)N(CCCCCCCCCCCCCCCCC)C2=CC=C(C=C2)O)C3=CC=C(C=C3)O</chem> |
| 63.....     | <chem>CC(C1=CC=C(C=C1)N(CCCCCCCCCCCCCCCCC)C2=CC=C(C=C2)O)C3=CC=C(C=C3)O</chem> |
| 64.....     | <chem>CC(C1=CC=C(C=C1)N(CCCCCCCCCCCCCCCCC)C2=CC=C(C=C2)O)C3=CC=C(C=C3)O</chem> |
| 65.....     | <chem>CC(C1=CC=C(C=C1)N(CCCCCCCCCCCCCCCCC)C2=CC=C(C=C2)O)C3=CC=C(C=C3)O</chem> |
| 66.....     | <chem>CC(C1=CC=C(C=C1)N(CCCCCCCCCCCCCCCCC)C2=CC=C(C=C2)O)C3=CC=C(C=C3)O</chem> |
| 67.....     | <chem>CC(C1=CC=C(C=C1)N(CCCCCCCCCCCCCCCCC)C2=CC=C(C=C2)O)C3=CC=C(C=C3)O</chem> |
| 68.....     | <chem>CC(C1=CC=C(C=C1)N(CCCCCCCCCCCCCCCCC)C2=CC=C(C=C2)O)C3=CC=C(C=C3)O</chem> |
| 69.....     | <chem>CC(C1=CC=C(C=C1)N(CCCCCCCCCCCCCCCCC)C2=CC=C(C=C2)O)C3=CC=C(C=C3)O</chem> |
| 70.....     | <chem>CC(C1=CC=C(C=C1)N(CCCCCCCCCCCCCCCCC)C2=CC=C(C=C2)O)C3=CC=C(C=C3)O</chem> |
| 71.....     | <chem>CC(C1=CC=C(C=C1)N(CCCCCCCCCCCCCCCCC)C2=CC=C(C=C2)O)C3=CC=C(C=C3)O</chem> |
| 72.....     | <chem>CC(C1=CC=C(C=C1)N(CCCCCCCCCCCCCCCCC)C2=CC=C(C=C2)O)C3=CC=C(C=C3)O</chem> |
| 73.....     | <chem>CC(C1=CC=C(C=C1)N(CCCCCCCCCCCCCCCCC)C2=CC=C(C=C2)O)C3=CC=C(C=C3)O</chem> |
| 74.....     | <chem>CC(C1=CC=C(C=C1)N(CCCCCCCCCCCCCCCCC)C2=CC=C(C=C2)O)C3=CC=C(C=C3)O</chem> |
| 75.....     | <chem>CC(C1=CC=C(C=C1)N(CCCCCCCCCCCCCCCCC)C2=CC=C(C=C2)O)C3=CC=C(C=C3)O</chem> |

| Example No. | Additive Structure |    |
|-------------|--------------------|----|
| 44          |                    | 5  |
| 45          |                    | 10 |
| 46          |                    | 15 |
| 47          |                    | 20 |
| 48          |                    | 25 |
| 49          |                    | 30 |
| 50          |                    | 35 |

This application is a continuation-in-part of our application Serial No. 119,752, filed October 5, 1949, now abandoned.

We claim:

1. A water-resistant thickened lubricant of good temperature susceptibility properties consisting essentially of a mineral lubricating oil of lubricating viscosity, an amount of an inorganic gelling agent to impart a grease-like consistency to the oil upon addition thereto, and an oil-soluble, water-insoluble, surface active alkyl alkylol imidazoline having the formula



where R is an alkylol group and R' is selected from the group consisting of alkyl and alkylene groups, said compound being in an amount to impart stability against deterioration by water.

- 5 2. A water-resistant thickened lubricant of good temperature susceptibility properties in accordance with claim 1, wherein R is hydroxyethyl.

3. A water-resistant thickened lubricant of good temperature susceptibility properties in accordance with claim 1, wherein R' is undecyl.

4. A water-resistant thickened lubricant of good temperature susceptibility properties in accordance with claim 1, wherein R' is heptadecyl.

- 15 5. A water-resistant thickened lubricant of good temperature susceptibility properties in accordance with claim 1, wherein R' is heptadecenyl.

6. A water-resistant thickened lubricant of good temperature susceptibility properties in accordance with claim 1, wherein the imidazoline is:



7. A water-resistant thickened lubricant of good temperature susceptibility properties in accordance with claim 1, wherein the imidazoline is:



8. A water-resistant thickened lubricant of good temperature susceptibility properties in accordance with claim 1, wherein the imidazoline is:



### Tall oil HC residue

9. A water-resistant thickened lubricant of good temperature susceptibility properties in accordance with claim 1, wherein the imidazoline is:



**References Cited in the file of this patent**

UNITED STATES PATENTS

- 2,531,440 Jordan ----- Nov. 28, 1950  
2,554,222 Stross ----- May 22, 1951